

June 11, 1946.

R. F. RENNIE

2,402,084

CONTINUOUS REDUCTION OF MOLYBDENUM COMPOUNDS

Filed Jan. 7, 1943

2 Sheets-Sheet 1



INVENTOR

R. F. RENNIE

BY *J. M. Reinhartz*  
ATTORNEY

June 11, 1946.

R. F. RENNIE

2,402,084

## CONTINUOUS REDUCTION OF MOLYBDENUM COMPOUNDS

Filed Jan. 7, 1943

2 Sheets-Sheet 2



**INVENTOR**

INVENTOR  
*R. F. RENNIE*

BY *J. M. Greenhaw*  
ATTORNEY

## UNITED STATES PATENT OFFICE

2,402,084

CONTINUOUS REDUCTION OF  
MOLYBDENUM COMPOUNDS

Robert Fredrik Rennie, Lake Forest, Ill., assignor  
to Westinghouse Electric Corporation, East  
Pittsburgh, Pa., a corporation of Pennsylvania

Application January 7, 1943, Serial No. 471,604

15 Claims. (Cl. 75—84)

1

This invention relates to the manufacture of molybdenum, and more particularly to a method of continuously reducing compounds of molybdenum, such as the trioxide and ammonium molybdate, for that purpose.

The principal object of my invention, generally considered, is in shortening and otherwise improving on the manufacture of molybdenum, starting with a reducible compound, avoiding slow reduction due to keeping the reaction temperature low, and continuously moving the compound through a furnace in a direction opposite to that of the reducing gas.

Another object of my invention is the reduction of molybdenum trioxide, or other reducible compound, to molybdenum, while continuously moving the same in a direction opposite to the flow of the reducing gas.

A further object of my invention is the reduction of a molybdenum compound to molybdenum, by moving it in a furnace continuously through heat zones of increasing temperatures, while passing reducing gas through said furnace in a direction opposite to that of said movement, at the same time stepwise increasing by effective concentration the strength of said reducing gas, to improve the quality of the metal produced and in order to avoid a runaway reaction.

Other objects and advantages of the invention, relating to the particular features and steps of the process, will become apparent as the description proceeds.

Referring to the drawings:

Figure 1 is a vertical longitudinal sectional view, with parts in elevation and parts shown diagrammatically, of a furnace and associated apparatus for reducing molybdenum compounds to molybdenum.

Figure 2 is a vertical, longitudinal, sectional view, with parts in elevation and parts shown diagrammatically, of another embodiment of a furnace and associated apparatus for practicing my invention.

Figure 3 is a view similar to Fig. 2, except a furnace part is shown fragmentarily in elevation, and the loading end of the furnace is open while the unloading mechanism is shown in engagement with boats for the purpose of removing them from the furnace.

In my copending application, Serial No. 413,118, filed October 1, 1941, now Patent No. 2,385,843, dated October 2, 1945, I have disclosed a method of reducing ammonium molybdate to molybdenum, making use of some of the ammonia generated during the breaking down of the molyb-

2

date for reduction purposes, and diluting the hydrogen used in the main reducing action with steam in order to slow down the reaction where necessary and avoid the formation of imperfect metal. This process is an improvement over that previously employed, but is not continuous in that the molybdate is introduced into the furnace and the reducing atmosphere and temperature varied as desired until it is changed to molybdenum, whereupon it is withdrawn.

In my copending application, Serial No. 458,106, filed September 12, 1942; I have disclosed a method of reducing molybdenum trioxide to molybdenum, which is similar to that of reducing ammonium molybdate to molybdenum, as disclosed in my application above-mentioned, except that the material is preferably granulated before reduction and I suggested using reducing agents other than hydrogen, it of course being understood that in the reduction of the trioxide there is no ammonia inherently available for reducing purposes.

The present invention is an improvement over the above-mentioned processes for stationary reduction of molybdenum compounds by various reducing gases, in that I propose to move the charge to be reduced forward at constant speed into zones of increasing temperature and in a direction opposite to that of the flow of the reducing gas, whereby said gas may be introduced when in its most concentrated or highly reducing condition, and reduced in strength, not only by the steam evolved during the reduction process, but also by the addition of desired amounts of steam along the length of the furnace, thereby avoiding a runaway reaction at the beginning of the reduction process, and improving the quality of the metal which is produced.

Since the time-temperature schedules for such a reduction have been worked out for stationary reductions, as described in the aforementioned pending applications, I have correspondingly arranged the speed with which the charge moves forward and the length of the different temperature zones so as to substantially conform with said schedules, the difference being necessitated by the fact that the control is by the strength of the reducing agent, temperature, length of heating zones, and the speed of movement of the charge therethrough, rather than by varying the flow of hydrogen or other reducing gas and the amount of diluting material during an increase in temperature of the reduction furnace.

Before this improvement was introduced, there was some difficulty when one tried to decide what

flow of hydrogen, or other reducing gas, to use. If the reduction tube was fed with the amount of hydrogen that is needed in the end zone, it would cause a too violent reaction in the zones of lower temperature, or those near where the reaction is beginning. If the furnace was fed with the amount of hydrogen that is wanted at the beginning of the reduction process, the end zone would have to be made impractically long to give complete reduction.

For this reason, continuous processes for reduction of molybdenum compounds up until now have been split into two parts, the end point of the first part being molybdenum dioxide, or a mixture of molybdenum dioxide and molybdenum trioxide.

This invention, therefore, supplies a practical solution for a one step reduction of molybdenum compounds to molybdenum by a continuous process. I propose to feed the reduction tube with the hydrogen, or other reducing gas, necessary for speedy complete reduction in the end zone, and at different points admit controlled amounts of steam, or other diluting agent, into the reduction tube to slow down the reaction where necessary and prevent the formation of imperfect metal.

Referring now to the drawings in detail, like parts being designated by like reference characters, and first considering the embodiment of my invention illustrated in Fig. 1, there is shown a furnace 11 consisting of a preferably slightly inclined reduction tube 12, which may be of about 4" internal diameter and formed of relatively refractory material, such as nichrome. This tube may be covered with suitable insulating material 13, in turn enclosed in a sheet metal envelope 14 and heated in any desired manner, as by means of resistance wires 15, 16, and 17, respectively, controlled by rheostats 18, 19 and 21 to provide three heating zones, respectively designated as 22, 23 and 24.

The windings, insulation, and other characteristics of the furnace are such that the heating zone 22 may be maintained at about 400° C., the zone 23 at about 630° C., and the zone 24 at about 1075° C. The furnace and accessories are desirably held in position as by means of supports 25. The left hand end of the furnace has a section desirably cooled by a water jacket 26 and provided with an outlet pipe 27 for the excess hydrogen, steam and/or ammonia, or other reagent used during the process. It is closed by a hinged door or cap 28, desirably including power means for pushing the molybdenum compound through the furnace, such as an air or water cylinder 29 and piston 31 for operating a rod 32 and associated pusher element 33. This or other suitable means may be used for moving the containers on boats 34, of the molybdenum compound to be reduced, at uniform speed from the left hand or inlet end of the furnace to the right hand or outlet end. The door or cap 28 may be secured in place by locking means 35, and provided with a chain 30 to a counterweight and lifting apparatus (not shown).

The outlet end of the furnace is provided with a section cooled by a water jacket or like means 36 and provided with a pipe 37 for introducing a supply of hydrogen or other reducing gas. The extreme end of the cooling section 38 of the tube 12 is closed by a hinged lid or door 39, provided with a suitable latch or locking device 41. Means are provided for introducing desired

amounts of water, or other diluting agent, along the length of the tube 12, said means in the present embodiment comprising pipes 42, 43 and 44. Water for these pipes is supplied from a reservoir 45 kept in the desired level as by means of a float valve (not shown) in the water supply pipe 46. The flow of the water from the reservoir to the pipes 42, 43 and 44 is controlled by valves 47, 48 and 49, respectively, admitting water through gaged capillary tubes 51, 52 and 53 and transparent connections 54, 55 and 56, permitting observation of the flow of water.

The hydrogen or other reducing gas supplied passes to the reduction tube at a desirably continuous rate being, however, naturally steadily attenuated during the reaction process by steam and/or other reaction product, with the excess withdrawn from pipe 27 for reclamation after the condensation of any steam therefrom.

I will now describe a preferred reduction schedule of molybdenum trioxide to molybdenum, preferably using hydrogen on granulated material, the manufacture of which has been described in my application, Serial No. 458,106, previously referred to, although I do not wish to be limited to the use of such material, as ammonium molybdate and other reducible molybdenum compounds may be handled in a similar manner. Instead of hydrogen, mixtures thereof such as "Endogas" (which is mainly a mixture of hydrogen and carbon monoxide, diluted with nitrogen) and water gas, and other reducing agents such as carbon monoxide, ammonia, and reducing mixtures, as referred to in said application, Serial No. 458,106, may be employed. It will also be understood that other diluting agents such as nitrogen and carbon dioxide, as referred to in said application, may be employed instead of, or admixed with, steam or with each other. The schedule disclosed is merely illustrative and changes may be made within the broad scope of my invention.

The preferably granulated molybdenum trioxide ( $MoO_3$ ) is placed in boats 34, desirably formed of refractory metal such as nickel, preferably about 2 kilograms per boat, the material being spread out in the boats to expose as much surface as possible.

The loaded boats may be first introduced into the cool or left hand end portion of the tube 12, after opening the cap or door 28, a sufficient number of boats being placed in front of the pusher element 33 so that the process may be continuous for a desired number of hours without shutting off the flow of hydrogen, or other reducing gas, and replenishing the supply of material to be reduced. After insuring that both doors 28 and 39 are closed and that cooling water is circulating through the water jackets, the hydrogen supply is turned on, as by opening the valve 57, to flush out the air in the tube 12 in order to insure that no explosion will occur when the furnace is brought to a higher temperature.

The electric current is then turned on to the resistance wires 15, 16 and 17, or other heating source applied, until the zones of the furnace reach the desired temperatures, as may be indicated by suitable pyrometers (not shown). That is, the temperature in the zone 22 controlled by wire 15 is desirably 400° C., that in zone 23 controlled by wire 16 is desirably 630° C., and that in zone 24 controlled by wire 17 is desirably 1075° C. The flow of water to the pipes 42, 43 and 44 is regulated so that we desirably get about 3 cc. per minute from the pipe 42, about 9 cc.

per minute from the pipe 43, and about 3 cc. per minute from the pipe 44.

The purpose is to admit enough water by pipe 43 to make the reaction to molybdenum dioxide, or intermediate reduction product, come to a standstill, with approximately 100% of that product at the point of admission of pipe 43. Enough water is to be admitted by pipe 44 to slow the reaction from the molybdenum trioxide, or starting product, sufficiently to prevent overheating and premature formation of imperfect metal. Compared with the stationary reduction described in the applications referred to, more than proportionate amounts of steam must be added because at the point of entry of pipe 43 there will be about 100% excess of hydrogen, and at the point of entry of pipe 44 there will be about 300% excess of hydrogen. This continued addition of steam during the process of reduction desirably coarsens the metal powder produced. This explains the reason for the steam inlet pipe 42, which is not to control the speed of reduction, but to control particle size of reduced metal. In certain cases, however, it may not be necessary to add any water by this pipe 42, or the proportion of water at this point may be varied, depending on the progress of the reduction as determined by experience.

At the same time air is admitted to the end pipe 58, as by means of a suitable control valve (not shown), to cause the pusher element 33 to start uniform movement of the boats 34 through the various zones of the furnace at a rate of speed calculated to leave said boats in zone 22 for about one hour, in zone 23 for about 2 1/4 hours, and in zone 24 for about 3 1/2 hours. The lengths of said zones are thus made proportionate to the times in which the boats are to remain therein, that is, in the ratio of 1:2 1/4:3 1/2.

The operation, therefore, starts at about 400° C. with the hydrogen or other reducing gas diluted with a maximum amount of steam, or other diluting agent, not only on account of the introduction of water, but also because of the formation of water by reaction of hydrogen with the oxygen of the molybdenum trioxide, or other oxygen compound, as said agent passes along the reducing tube from right to left. This reducing action by the hydrogen, or other reducing gas, starts the reduction of molybdenum trioxide, or other compound, toward a lower oxidation product, such as the dioxide, avoiding by dilution a runaway reaction at undesired high temperatures and the production of imperfect metal.

Finally the boats successively reach the next zone where they are heated to a temperature of about 630° C., in a reducing atmosphere more concentrated than that in the zone 22, because there is not only less water admitted in this zone, but there has been less impoverishment of the reducing gas. In this second zone the reduction to molybdenum dioxide is substantially completed so that upon reaching the zone 24, of the higher temperature of about 1075° C., the still more concentrated reducing atmosphere may be safely employed without danger of a runaway reaction or the development of imperfect metal.

If molybdenum trioxide is reduced in this manner, the reaction is in accordance with the following equations:



The above equations were developed from the following matter taken from Gmelin, Handbuch der anorganischen Chemie, 8 Auflage.

1.  $\text{MoO}_3 \rightarrow \text{MoO}_2 + \frac{1}{2}\text{O}_2 - 38,700$  (p. 96)
2.  $\text{MoO}_2 \rightarrow \text{Mo} + \text{O}_2 - 142,800$  (p. 92) and
3.  $\text{H}_2 + \frac{1}{2}\text{O}_2 \rightarrow \text{H}_2\text{O} + 68,400$  from Handbook of Chemistry and Physics, 21st edit., p. 1004. (Chemical Rubber Publishing Co.)

If other materials or other reducing gases are employed, the equations will be in accordance with those quoted in the applications, Serial Nos. 413,118 and 458,106, previously referred to.

The foregoing reduction process may be summarized by the following table:

| Hours      | O'clock            | Furnace temp. |                                                                                                                                              |
|------------|--------------------|---------------|----------------------------------------------------------------------------------------------------------------------------------------------|
| 1.....     | 8:00 to 9:00.....  | 400           | 50 cu. ft. of $\text{H}_2$ per hr. + 15+ cc. $\text{H}_2\text{O}$ per min. <sup>1</sup>                                                      |
| 2 1/4..... | 9:00 to 11:15..... | 630           | 50 cu. ft. of $\text{H}_2$ per hr. + 12+ cc. $\text{H}_2\text{O}$ per min. Reduction to $\text{MoO}_2$ nearly complete. <sup>1</sup>         |
| 3 1/4..... | 11:15 to 2:45..... | 1,075         | 50 cu. ft. of $\text{H}_2$ per hr. + from 3+ cc. to no $\text{H}_2\text{O}$ per min. Remainder of $\text{MoO}_2$ reduced to Mo. <sup>1</sup> |

<sup>1</sup> The flow of  $\text{H}_2$ , starting at 50 cu. ft. per hr. at exit end of furnace, is continually reduced to a variable extent due to combining with the O of the  $\text{MoO}_3$  and  $\text{MoO}_2$  during the process.

From the foregoing it will be seen that I have shortened the schedule to 6 1/4 hours, from the 9 hour schedule of the applications previously referred to. I have, as in said earlier applications, also provided for the elimination of clinkers and/or cones and made it possible to reduce from a high oxidation form, such as the trioxide, directly to the metal in one continuous process, that is, pushing the boats of oxide in one end of a furnace and withdrawing them from the other end, while maintaining a continuous flow of reducing and diluting materials through said furnace. At the same time, I provide for salvage of any unused hydrogen or other reducing gas.

It will, of course, be understood that the continuous time of any process, prior to removal of the reduced metal and re-charging with oxide or other compound depends on the length of the reduction tube, as in the embodiment described the pusher element 33 can operate only until the charge associated therewith reaches the end of the tube or outlet door 39 thereof. It is, therefore, believed desirable that the inlet end of the furnace, or that cooled by the water jacket 26, be of a length corresponding with the intermediate or heated portion thereof, and that the outlet end, or that cooled by the water jacket 36, be of a corresponding length, so that a charge of boats equal in length to the heated portion of the tube, that is the portion consisting of the zones 22, 23 and 24, may be started in the cool left hand end of the furnace and the operation continued until completed, when the entire charge will have been moved to the outlet end. Thereupon the hydrogen or reducing gas supply may be shut off, the heating current terminated, the flow of water or other diluting agent stopped and, when the furnace is sufficiently cool to avoid undesired oxidation of the reduced metal, the door 39 may then be opened and the charge of metal removed, after which the door 28 may be opened and a new charge of oxide, or other reducible molybdenum compound, introduced and the process repeated.

Referring now to the embodiment of my invention illustrated in Figs. 2 and 3, there is frag-

mentarily shown a furnace 11<sup>a</sup>, which may be identical with the furnace 11 of the preceding embodiment insofar as the central or heating section is concerned. However, the left hand or loading end of the inclined reduction tube 12<sup>a</sup> of the furnace of the present embodiment, has a section that is cooled by water jacket 26<sup>a</sup> and provided with an outlet pipe 27<sup>a</sup> for excess hydrogen, steam and/or ammonia or other reagent used during the process, and said section need not be as long as the furnace or heating section for reasons which will be explained.

In the present instance the loading end of the tube 12<sup>a</sup> is closed by a door or cap 28<sup>a</sup>, including power means for pushing the molybdenum compound through the furnace, such as, for example, an hydraulic cylinder 29<sup>a</sup>, piston 31<sup>a</sup>, operating a rod 32<sup>a</sup>, and associated pusher element 33<sup>a</sup>. This or other suitable means may be used for moving the containers or boats 34<sup>a</sup> of the molybdenum compound at uniform speed, from the left hand or inlet end of the furnace to the right hand or outlet end. The door or cap 28<sup>a</sup> is, in the present instance, hinged at its lower end rather than at its upper end and normally secured in place by locking means 35<sup>a</sup>. As in the preceding instance, the cylinder 29<sup>a</sup> is provided with a chain 30<sup>a</sup> to a counterweight and lowering apparatus (not shown).

The outlet end of the furnace is provided with a section, cooled by water jacket or like means 36<sup>a</sup> and provided with a pipe 37<sup>a</sup> for introducing a supply of hydrogen or other reducing gas. The extreme end of the cooling section 38<sup>a</sup> of the reduction tube 12<sup>a</sup> is closed by a cap or lid 39<sup>a</sup>, provided with suitable latch or locking device 41<sup>a</sup>. The cooling section 38<sup>a</sup> of the reduction tube 12<sup>a</sup> is in this instance formed in two sections which may be separated as in Fig. 2, or connected as in Fig. 3, by closing or opening the gate valve 61.

The cap 39<sup>a</sup> is provided with an aperture containing a sleeve element 62 and hooked rod 63, controlled by a handle 64, so that they are adapted to be reciprocated and turned at will. They may be moved toward the entrance end of the reduction tube when the gate valve 61 is open, as in Fig. 3, and turned so that the hooked end portion 66 of the rod 63 engages one or more of the boats 34<sup>a</sup> to pull it, or them, to the right hand position shown in Fig. 2, whereupon the gate valve may be closed; the cap 39<sup>a</sup> and its associated sleeve and rod removed, and the boats taken out of the furnace. The sleeve 62 is desirably provided with a collar or flange 65 which is adapted to engage the forward or right hand end of a boat 34<sup>a</sup> to tell the operator when to turn the handle 64 so that the hooked end portion 66 thereof will connect with the boat or boats 34<sup>a</sup> nearest the exit end of the furnace.

The hydrogen supply pipe 67 is desirably provided with a branch 68 controlled by a valve 69 so that the extreme right hand section of the reduction tube, or that beyond the gate valve 61, may, prior to opening said valve to resume the reducing operation, be flushed out with hydrogen so that when said gate valve is opened an explosive mixture will not be formed. During the flushing operation the air is exhausted through pipe 71 controlled by valve 72.

The operation of the embodiment of my invention illustrated in Figs. 2 and 3 may be as follows:

The loaded boats of the reducible compound, such as the granulated trioxide, may be first introduced into the cool or left hand end portion

of the tube 12<sup>a</sup> after dropping the cap or door 28<sup>a</sup>. Any convenient number of boats are placed in front of the pusher element 33<sup>a</sup>. When the door 28<sup>a</sup> is open, the valve 73 in the hydrogen exhaust pipe 27<sup>a</sup> is closed as by releasing the spring actuated stem 74 thereof by swinging the adjustable pusher element 70 of the operating arm 75 from engagement therewith. The arm 75 is integral with or connected to the door 28<sup>a</sup> so as to swing therewith.

At the same time the valve 76 is opened, as by release of its spring actuated stem 77 by disengagement of the arm-carried adjustable pusher element 80, to increase the supply of gas to the pipe 78 to change the pilot light 79 issuing therefrom to a relatively long flame 81 and thereby ignite the issuing hydrogen, or other reducing gas 82, and prevent the formation of an explosive mixture.

When the furnace is open, as represented in Fig. 3, then the charge of boats 34<sup>a</sup> may be introduced, as by pushing them in along a loading plate 83 by means of a pusher element 84, after which the door 28<sup>a</sup> is closed as in Fig. 2, automatically reducing the flame 81 to the pilot light 79 and opening the reducing gas exhaust pipe valve 73 by bringing the operating arm 75 into engagement therewith.

The hydrogen, or reducing gas supply is then turned on, the furnace brought up to temperature, and the reducing action started as described in connection with the embodiment of Fig. 1. The hydraulic cylinder or other operating means pushes the boats 34<sup>a</sup> a desired distance into the furnace, whereupon the pusher element 33<sup>a</sup> may be withdrawn, the filling end of the furnace opened, and some more boats placed therein, as illustrated in Fig. 3.

This pushing and withdrawing operation is repeated until it is estimated that the boats at the head or right hand end of the line are coming close to the gate valve 61. Said gate valve 61 is then opened, the hooked rod 63 moved from the position shown in Fig. 2 to that shown in Fig. 3 and turned to engage one or more of the boats 34<sup>a</sup> and pull them to the extreme right hand position shown in Fig. 2. The gate valve 61 is then closed, the exit cap 39<sup>a</sup> and its hooked rod 63 removed therefrom and the captured boats taken out of the furnace. The cap 39<sup>a</sup> and rod 63 are reapplied to the furnace as in Fig. 2, the outer section or that to the right of the valve 61 flushed out with hydrogen, the valves 69 and 72 closed, the gate valve 61 opened.

It will be understood that the reducing operation may be continued uninterruptedly during the operation of the loading or unloading of the furnace. The short stoppage time taken for loading is allowed for as part of the reduction time, the time taken for unloading, however, not affecting the reduction time because during the unloading operation the piston 31<sup>a</sup> may operate and continue to push the boats from left to right in the reduction tube.

In brief, during continuous operation the following steps will preferably occur:

1. Pusher element 32<sup>a</sup> moved from position in Fig. 2 to extreme left position.
2. Door 28<sup>a</sup> moved from position in Fig. 2 to that of Fig. 3.
3. Charge introduced as shown in Fig. 3.
4. Door 28<sup>a</sup> closed and pusher element 33<sup>a</sup> restarted by operation of hydraulic cylinder.
5. Gate valve 61 opened and hooked member moved from position in Fig. 2 to that of Fig. 3 to

engage one or more boats and withdraw same to extreme right hand position as shown in Fig. 2.

6. Gate valve 61 closed.
7. Cap 38<sup>a</sup> and hooked rod 63 removed.
8. Boats in outer end 38<sup>a</sup> or reduction tube withdrawn therefrom.
9. Cap 38<sup>a</sup> and hooked rod 63 reapplied.
10. Outer section 38<sup>a</sup> of reduction tube flushed out with hydrogen or other reducing gas.
11. Gate valve 61 opened, completing the cycle of operations.

It will thus be seen that my reduction process may be continuous for a predetermined period, when using the apparatus of Fig. 1 or continuous for an indefinite period, when using the apparatus illustrated in Figs. 2 and 3. It will also be understood that the description of the apparatus of Fig. 2 is to be supplemented by the description of the apparatus of Fig. 1, insofar as the details of the furnace or heating portion of the apparatus and the reduction schedule is concerned. The essential difference between the two operations is that in connection with the second embodiment the loading piston will periodically move back to accommodate charges, that is, move at a substantially continuous and uniform rate punctuated only by the brief loading intervals, and the reduced metal will be withdrawn without stopping the furnace, while in the first embodiment the charge is started at the loading end and pushed on through to the unloading end without opening the furnace or stopping the movement of the boats in any manner.

It will be understood that, as in my prior application, Serial No. 458,106, no water or other diluting agent need be employed if a sufficiently weak reducing gas, such as ammonia or Endogas, is initially employed, as the heat generated during the reaction is considerably less, especially in my present improved process which inherently provides for a weaker reducing action at the start because of the travel of the reducing gas in a direction opposite to that of the compound being reduced and the continuous dilution of the gas by the gaseous product of reduction. In the reduction of ammonium molybdate, making use of ammonia generated during the reducing action, the hydrogen obtained by the cracking of the ammonia is diluted with uncracked ammonia. It will also be understood that if desired my process may be controlled by pressure as described in connection with my co-pending application, Serial No. 458,106.

Although preferred embodiments of my invention have been disclosed, it will be understood that modifications may be made within the spirit and scope of the broad idea.

I claim:

1. The method of producing molybdenum from a reducible compound thereof, comprising moving said compound through a furnace, passing a reducing gas through said furnace in a direction opposite to that of the movement of said compound, and introducing gas inert to said compound into said furnace intermediate the ends thereof, to slow down the initial reaction until the reduction is partially effected.

2. The method of producing molybdenum from a reducible compound thereof, comprising moving said compound through a furnace from a relatively low temperature zone into one of higher temperature, passing a reducing gas through said furnace, and diluting said reducing gas by introducing an inert gas into said furnace intermediate the ends thereof in order to slow down the initial reaction until the reduction is partially effected.

the initial reaction until reduction is partially effected.

3. The method of producing molybdenum from a reducible compound thereof, comprising moving said compound through a furnace from a relatively low temperature zone into one of higher temperature, passing a reducing gas through said furnace in a direction opposite to that of the movement of said compound, and diluting said reducing gas by introducing an inert gas into said furnace intermediate the ends thereof in order to slow down the initial reaction until reduction is partially effected.

4. The method of producing molybdenum from a reducible compound thereof, comprising moving said compound through a furnace from a relatively low temperature zone into one of higher temperature, passing hydrogen through said furnace, and diluting said hydrogen by introducing an inert gas into said furnace intermediate the ends thereof in order to slow down the initial reaction until reduction is partially effected.

5. The method of producing molybdenum from a reducible compound thereof, comprising moving said compound through a furnace from a relatively low temperature zone into one of higher temperature, passing a gaseous reducing mixture through said furnace, and diluting said mixture with inert gas intermediate the ends of said furnace in order to slow down the initial reaction until reduction is partially effected.

6. The method of reducing molybdenum trioxide comprising moving it through a furnace, passing hydrogen through said furnace in a direction opposite to that of the movement of said trioxide, and diluting said hydrogen with steam intermediate the ends of said furnace in order to slow down the initial reaction until the reduction is partially effected.

7. The method of reducing ammonium molybdate comprising moving it through a furnace, passing hydrogen through said furnace in a direction opposite to that of the movement of said molybdate, and diluting said hydrogen with steam intermediate the ends of said furnace in order to slow down the initial reaction until reduction is partially effected.

8. The method of reducing molybdenum trioxide comprising moving it through a furnace from a relatively low temperature zone into one of higher temperature, passing hydrogen through said furnace in a direction opposite to that of the movement of said trioxide, and diluting said hydrogen with steam intermediate the ends of said furnace in order to slow down the initial reaction until reduction is partially effected.

9. The method of reducing ammonium molybdate comprising moving it through a furnace from a relatively low temperature zone into one of higher temperature, passing hydrogen through said furnace in a direction opposite to that of the movement of said molybdate, and diluting said hydrogen with steam intermediate the ends of said furnace in order to slow down the initial reaction until reduction is partially effected.

10. The method of producing molybdenum from a reducible compound thereof comprising moving said compound through a furnace from a relatively low temperature zone into one of higher temperature, and passing a gaseous mixture, containing a large enough proportion of hydrogen and carbon monoxide to effect reduction of said compound, through said furnace in a direction opposite to that of the movement of said compound, and introducing gas inert to said com-

pound into said furnace intermediate the ends thereof, to slow down the initial reaction until the reduction is partially effected.

11. The method of reducing molybdenum tri-oxide comprising moving it in a furnace through and from a heat zone of about 400° C. into and through one of about 630° C., and then into and through one of about 1075° C., while passing hydrogen through said furnace in a direction opposite to that of the movement of said tri-oxide, and diluting the hydrogen in said furnace at a distance from its place of admission, and in at least some of said heat zones, in order to slow down the reaction until reduction is partially effected.

12. The method of reducing molybdenum tri-oxide comprising moving it successively into and through zones heated, respectively, to 400°, 630° and 1075° C., passing hydrogen through said furnace in a direction opposite to that of the movement of said trioxide, and diluting said hydrogen with steam at various points along said furnace, in order to effect a slowing down of the reaction at the earlier stages until reduction is sufficiently effected to avoid excessive generation of heat by the reducing action.

13. The method of reducing molybdenum tri-oxide comprising moving it successively into and through zones in a reduction tube of about four inches internal diameter and heated respectively to 400°, 630° and 1075° C., passing hydrogen at the rate of about 50 cu. ft. per hour through said furnace in a direction opposite to that of the movement of said trioxide, and diluting said hydrogen with direct additions of steam in each heat zone, in order to effect a slowing down of the reaction in the earlier stages, until reduction is sufficiently effected to avoid excessive generation of heat by the reducing action.

14. The method of producing molybdenum from a reducible compound thereof comprising placing said compound in containers, introducing some of said containers in front of a pusher element in the reduction tube of a furnace, closing said tube, starting said pusher element to move said containers at a uniform rate of speed

through said tube, passing a reducing gas through said tube in a direction opposite to that of the movement of said compound, introducing inert gas into said furnace intermediate the ends thereof to slow down the initial reducing action until the reduction is partially effected, pulling a desired number of said containers, after reduction of the compound therein, to the opposite extreme end of said tube, closing off said extreme end portion of said tube from the main portion thereof, opening said extreme end portion of said tube, withdrawing the captured containers, closing said extreme end portions, flushing out said closed end portion of said tube with reducing gas, reconnecting said closed end portion with the main portion of said tube, and repeating said steps whereby the reducing operation may be continuous.

15. The method of producing molybdenum from the trioxide comprising placing said tri-oxide in containers, introducing some of said containers in front of a pusher element in a cooled end portion of the reduction tube of a furnace, closing said tube, starting said pusher element to move said containers at a uniform rate of speed through zones in said tube heated, respectively to 400°, 630° and 1075° C., passing hydrogen through said tube in a direction opposite to that of the movement of said trioxide, diluting said hydrogen with steam at various points along said tube, to slow down the initial reducing action until the reduction is partially effected, pulling a desired number of said containers, after reduction of the trioxide therein, to the opposite extreme end of said tube, closing off said extreme end portion of said tube from the main portion thereof, opening said extreme end portion of said tube, withdrawing the captured containers, closing said extreme end portion, flushing out said closed end portion of said tube with hydrogen, reconnecting said closed end portion with the main portion of said tube, and repeating said steps whereby the reducing operation may be continuous.

ROBERT FREDRIK RENNIE.